

# United States Patent [19]

Nishino

[11] 3,841,874

[45] Oct. 15, 1974

[54] **METHOD FOR IMPROVING THE PHOTOGRAPHIC CHARACTERISTICS OF VESICULAR PHOTOGRAPHIC MATERIALS**

[75] Inventor: **Akio Nishino**, Los Gatos, Calif.

[73] Assignee: **Xidex Corporation**, Sunnyvale, Calif.

[22] Filed: **Mar. 29, 1973**

[21] Appl. No.: **346,202**

## Related U.S. Application Data

[63] Continuation-in-part of Ser. No. 124,584, March 15, 1971, abandoned.

[52] **U.S. Cl.** ..... 96/27 R, 96/48 HD, 96/49.75, 96/91 R, 96/115 R

[51] **Int. Cl.** ..... G03c 5/04, G03c 5/18

[58] **Field of Search**... 96/49.75, 91 R, 91 N, 11 SR, 96/48 HD, 27 R

[56]

## References Cited

### UNITED STATES PATENTS

|           |         |              |             |
|-----------|---------|--------------|-------------|
| 2,911,299 | 11/1959 | Baril et al. | ..... 96/49 |
| 3,032,414 | 5/1962  | James et al. | ..... 96/49 |
| 3,108,872 | 10/1963 | McMahon      | ..... 96/49 |
| 3,120,437 | 2/1964  | Lindquist    | ..... 96/49 |

|           |         |                 |             |
|-----------|---------|-----------------|-------------|
| 3,143,418 | 8/1964  | Priest et al.   | ..... 96/49 |
| 3,149,971 | 9/1964  | Baril et al.    | ..... 96/49 |
| 3,498,786 | 3/1970  | Notley et al.   | ..... 96/49 |
| 3,615,476 | 10/1971 | Cossiers et al. | ..... 96/49 |
| 3,615,486 | 10/1971 | Delzenne        | ..... 96/49 |

## FOREIGN PATENTS OR APPLICATIONS

|         |         |               |               |
|---------|---------|---------------|---------------|
| 645,825 | 11/1950 | Great Britain | ..... 96/91 R |
|---------|---------|---------------|---------------|

*Primary Examiner*—Charles L. Bowers, Jr.  
*Attorney, Agent, or Firm*—Townsend and Townsend

[57] **ABSTRACT**

Improvement of photographic characteristics of vesicular film such as an increase in its speed and a reduction in its gamma by contact of film prior to exposure with an alkanol having up to about three carbon atoms. Equivalent results are obtained by contact with acetonitrile where the film's vehicle is a thermoplastic linear poly (hydroxy ether) polymer of an epihalohydrin and a dihydric phenol. In both cases where such treatment is followed by a second treatment with water an even greater improvement in photographic characteristics is obtained. Following treatment an equilibration period is required to permit solvent to be released from the film.

13 Claims, No Drawings

**METHOD FOR IMPROVING THE  
PHOTOGRAPHIC CHARACTERISTICS OF  
VESICULAR PHOTOGRAPHIC MATERIALS**

This is a continuation-in-part of copending U.S. Pat. application Ser. No. 124,584, filed Mar. 15, 1971 now abandoned.

This invention relates to vesicular film. More particularly it relates to the treatment of vesicular film to improve its photographic characteristics such as speed and gamma.

Previously it has been disclosed that the treatment of vesicular film with an aqueous bath in liquid or vapor phase at elevated temperatures prior to exposure and development will reduce the gamma or contrast of the film providing a longer grey scale without sacrificing other desirable photometric characteristics. While reducing the gamma the treatment also provides an increase in the photographic speed of the film; see for example, U.S. Pat. No. 3,149,971 to Baril, Jr., et al. issued Sept. 22, 1964.

The present invention is based upon the discovery that these improvements and others are not solely obtainable by treatment of the film with water. It has now been discovered that certain organic solvents in liquid or vapor phase provide similar benefits to vesicular film. Use of these newly discovered organic fluids have certain advantages over the previously disclosed water treatment. For example, in the present method treatment of vesicular film can be executed at ambient temperature whereas the prior art has required the use of elevated temperatures. Moreover, in the preferred embodiment of the present invention, and as will be illustrated hereinafter, the treatment is more effective and faster than the prior art methods.

In accordance with the present invention the photographic characteristics of vesicular film are improved by contacting the film prior to exposure with a fluid phase alkanol having up to about 3 carbon atoms for a time and at a temperature sufficient to increase the photosensitivity thereof.

In another aspect of the invention in which the vesicular film has as its vehicle a film forming thermoplastic linear poly (hydroxy ether) polymer of an epihalohydrin and a dihydric phenol, the photographic characteristics can be improved by contacting the film prior to exposure with fluid phase acetonitrile. In both aspects of the invention significant and substantial improvements are obtained by treatment with the organic fluids noted. However, where an even greater improvement is desired, a second treatment by contacting the film with water following the initial contact with the organic fluid will result in further improvements of the photographic characteristics of the film.

Following contact with the treating fluid an equilibration period is required before the film is ready for imaging exposure. Solvent that has been absorbed during treatment is released during this period.

The process of this invention is carried out simply by contacting the film with the selected organic solvent. This is usually accomplished by immersing the film in a liquid bath containing the solvent or in a zone containing solvent vapor as for example, above a heated liquid bath, and thereafter in a liquid water bath where the two-stage treatment is employed. The particular time and temperature employed during such contact will vary depending upon the nature of the vehicle used in the vesicular film and the type and extent of photo-

graphic improvement desired. Within broad limits, increasing the time of contact and/or temperature of the bath will increasingly enhance the effects of the treatment until the maximum improvement possible is reached. Otherwise, the limiting factor will be that point where the film is adversely affected by excessive heat and/or attack by the solvent. While any time and temperature relationship which will result in a discernible improvement is contemplated, excellent results to date have been obtained where the acetonitrile or alkanol fluid is maintained at a temperature of about 20°-60° C., preferably 20°-40° C. for about 1-100 seconds. These temperatures and times apply to the use of either a liquid bath treatment or treatment by vapor phase acetonitrile or alkanol. Where a vapor phase is generated above a liquid bath by heating the liquid bath, the liquid bath will generally be at a temperature higher than that desired in the vapor phase. Moreover, a vapor temperature gradient has been observed in such a situation with the vapor temperature decreasing as distance from the liquid bath surface was increased. Accordingly, in such a situation the film to be treated is passed through the appropriate vapor zone above the liquid having the desired temperature.

Where the second stage water treatment is employed, a temperature range of about 20°-90° C. for the water with a contact time of about 1-100 seconds will usually be highly effective. As noted above, the present invention has the advantage of producing the desired improvement at ambient temperature. A highly useful result can be obtained using a slightly warmed alkanol treatment in the range of 30°-40° C. followed by an ambient water treatment, with both steps being completed within a total contact time of one minute or less.

Following immersion, solvent is released from the film during an equilibration period. This may be conveniently accomplished by storing the film so that the vehicle surface is in communication with the ambient atmosphere for a sufficient time to permit substantial release of solvent. If no solvent is released prior to image-wise exposure, the effects of the treatment are generally not great, or the film may even be substantially photographically inoperative. Generally, release of as much solvent as possible is desired so as to approach zero solvent retention. Retention of less than about 1% solvent is a practical goal.

The conditions of storage will govern the precise time at which sufficient equilibration has occurred so that the benefits of the treatment are fully obtained. Usually, sufficient solvent release may be obtained with as little as 1/4 to 1/2 hour of equilibration with the ambient atmosphere. In most cases best results are obtained with about 6-48 hours of equilibration. Even longer periods may be beneficial in some cases.

The vesicular film formulations which may be subjected to the treatment of this invention are in general conventional and contain the usual elements found in a vesicular film; namely, a synthetic hydrophobic organic polymeric vehicle within which is dispersed a light-sensitive chemical which decomposes to give a gas. The vehicle and light-sensitive element are generally coated on a suitable support such as the polyethylene terephthalate known as Mylar. All vesicular films which have such a structure and composition are contemplated for treatment by the present process. Such vesicular film formulations may optionally contain the usual additives such as a surfactant dispersed through

the vehicle along with the light-sensitive element. Suitable surfactants are described in copending U.S. Pat. application Ser. No. 55,976, filed July 17, 1970 now abandoned but refiled as continuation-in-part in U.S. Pat. application Ser. No. 175,348, filed Aug. 26, 1971, now U.S. Pat. No. 3,779,768 and in copending U.S. Pat. application Ser. No. 54,011, filed July 10, 1970 now abandoned but refiled as continuation-in-part in U.S. Pat. application Ser. No. 251,826, filed May 9, 1972, now U.S. Pat. No. 3,779,774.

With respect to the alkanol solvents used in the present treatment, any suitable synthetic organic thermoplastic or thermosetting vehicle for vesicular film may be employed which may be highly linear or cross linked. The only limitation on the choice of vehicle to be treated is that the vehicle should be insoluble in the treating fluid at least under the conditions of the treatment so as to retain its physical integrity as a useful photographic film. Suitable vehicles that are resistant to lower alkanol solvents and which may be benefited by the present treatment include the diverse synthetic organic polymeric vehicles described in the prior art including the vinyl polymeric vehicles described in the above-referenced U.S. Pat. No. 3,149,971, as well as the organic polymeric vehicles disclosed in U.S. Pat. Nos. 3,032,414 and 3,161,511. These preferred synthetic organic polymers used as the vehicle provide a moisture stable image after exposure and development. Such synthetic polymeric vehicles are distinguished from the older, naturally occurring non-synthetic vesicular vehicle materials such as gelatin which do not provide a vesicular image that is as stable under high moisture conditions.

In the present invention two classes of synthetic polymeric vehicles have been shown to respond to the process in a highly effective manner. The first class of such vehicles is formed from a copolymer of a larger amount of a nitrile of the formula:



copolymerized with a minor amount of a hydroxy substituted acrylate of the formula:



in which X and Y are individually selected from hydrogen, methyl, and chlorine and Z is the alkylene-oxy group:



in which n is an integer from 2-4, m is an integer from 1-2 provided that when m is 2, n is 2, and further provided that a hydroxyl group is substituted for a hydrogen atom of Z.

Vehicles of this type are disclosed and claimed in copending U.S. Pat. application Ser. No. 72,913, filed Sept. 17, 1970. As disclosed in said application, outstanding results are obtained where the copolymer is formed from 80-96 weight percent of methacrylonitrile and about 4-20 weight percent of 2-hydroxy ethyl methacrylate.

The other type of vehicle preferred in the present invention is a thermoplastic linear poly (hydroxy ether)

polymer of an epihalohydrin and a dihydric phenol. Such vehicles are disclosed in copending U.S. Pat. application Ser. No. 866,753, filed Oct. 15, 1969, now U.S. Pat. No. 3,622,333, with a preferred species thereof being a polymer of epichlorohydrin and 2,2'-bis(p-hydroxy phenyl) propane. Specific examples of other types of vehicles which may be used in the present invention will be described in the working examples which follow.

- 10 The alkanol which is preferably used in the present process is methyl alcohol although the other alkanols having up to about 3 carbon atoms including ethyl alcohol, propyl alcohol, and isopropyl alcohol are also shown to be highly effective. Higher molecular weight alcohols such as butyl alcohol are generally less desirable and may require impractically longer treatment times and/or higher temperatures. As mentioned earlier, where the vesicular film vehicle is a linear poly (hydroxy ether) of the type disclosed in the above-referenced U.S. Pat. application Ser. No. 866,753, acetonitrile can be used to improve the photographic characteristics of the film in a comparable manner. Acetonitrile appears to be unique in combination with the poly (hydroxy ether) vehicle. Numerous attempts to employ solvents other than alcohols with this and other vehicles were unsuccessful in the present context.

Example I illustrates the typical preparation and treatment of a vesicular film in accordance with this invention and the manner for testing its photographic properties. The experimental work reported in the other examples generally followed the same procedure except where indicated otherwise.

#### EXAMPLE I

35 Vesicular films were prepared from the following formula:

| Function   | Component                 | Parts by Weight |
|------------|---------------------------|-----------------|
| Vehicle    | Eponol 55                 | 5               |
| Sensitizer | Andrews Diazo No. 9       | 0.3             |
| Surfactant | L-79                      | 0.04            |
| Surfactant | L-5202                    | 0.005           |
| Solvent    | Methyl ethyl ketone (MEK) | 8               |
| 45 Solvent | 2-Methoxy ethanol         | 16              |

50 Eponol 55 is a poly (hydroxy ether) made by Shell Chemical Company from epichlorohydrin and 2,2'-bis(4-hydroxyphenyl) propane, Bisphenol A. Andrews' Diazo No. 9 is Andrews Paper and Chemical Company's p-diazo-N,N-diethylaniline zinc chloride. L-79 and L-5202 are Union Carbide's silicone surfactants. These are among the optional additives for vesicular film mentioned previously.

55 The diazo compound was dissolved in 2-methoxyethanol to a 13 percent solids solution; to this stirring solution was added the L-79 in a 25 percent methoxyethanol solution and the L-5202 in a 10 percent 2-methoxyethanol solution. This mixture was then added to a stirring solution of the Eponol 55 in the remaining solvents. The complete solution was then coated onto strips of polyethylene terephthalate (Mylar) with a Bird applicator knife to give, after drying for 5 minutes at 105° C., films of 0.4 mil thickness. A vesicular film thus obtained was immersed for 60 seconds in ambient (22° C.) water and dried with tissue paper. A second film was immersed for 15 seconds in 85° C.

water and dried with tissue paper. A third film was immersed for 10 seconds in ambient (22° C.) methanol and a fourth film was immersed for 15 seconds in ambient methanol and dried similarly. Equilibration was accomplished in the ambient atmosphere in about 16 hours. The treated films were then given identical exposures of 60 seconds through a Kodak Photographic Step Wedge No. 3, 4 inches away from a 325 watt Hanovia Mercury vapor lamp 654A10 and then developed at 110° C. in a Canon Kalfile Developer 360VS. A fifth film, which was not treated, was also exposed and developed in like fashion. Projection density (*f* 4.5) was measured on a MacBeth Quantalog Densitometer Model TD205. Photographic characteristics of these films were as follows:

5

15

| Treatment                     | Visbl<br>Steps | Dmax | Dmin | Speed at |                  |
|-------------------------------|----------------|------|------|----------|------------------|
|                               |                |      |      | OD=1     | amma<br>Dmin+0.1 |
| None                          | 2              | 0.98 | 0.08 | —        | —                |
| 60 seconds<br>22° C. Water    | 2              | 1.71 | 0.07 | 4.74     | 0.19             |
| 15 seconds                    | 7              | 1.72 | 0.06 | 3.33     | 0.60             |
| 85° C. Water<br>10 seconds    | 7              | 1.74 | 0.08 | 3.48     | 0.60             |
| 22° C. methanol<br>15 seconds | 8              | 1.75 | 0.08 | 2.96     | 0.63             |
| 22° C. methanol               | 8              | 1.75 | 0.08 | 0.97     | 0.97             |

Ambient water did not significantly improve photographic characteristics over those for the untreated film. The ambient methanol treated samples showed greatly improved characteristics. These improved characteristics were matched only when the film was subjected to water at a substantially elevated temperature.

30

## EXAMPLE II

Vesicular films were prepared from the following formula:

35

| Function   | Component                     | Parts by Weight |
|------------|-------------------------------|-----------------|
| Vehicle    | Methacrylonitrile homopolymer | 2.5             |
| Sensitizer | Andrews Diazo No. 9           | 0.1             |
| Solvent    | Acetonitrile                  | 5               |
| Solvent    | 2-Methoxyethanol              | 6               |

40

The vehicle was prepared by emulsion copolymerization of methacrylonitrile and methacrylic acid in a 90/10 weight ratio. Disperse-Ayd No. 6 is a surfactant from Daniel Products Company. The diazo compound was dissolved in the DMF and to this stirring solution was added a solution of the Disperse-Ayd No. 6 in the THF. The combined solution was then added to the stirring solution of the vehicle in MEK. Film preparation was as described in Example I. A vesicular film thus obtained was immersed for 60 seconds in ambient (23° C.) water and dried with tissue paper. Another film was immersed for 60 seconds in ambient (23° C.) methanol and dried in like fashion. Equilibration was accomplished in the ambient atmosphere in about 1½ hours. The films were then exposed and developed as described in Example I, with the following results:

| Treatment                     | Visbl<br>Steps | Dmax | Dmin | Speed at |                  |
|-------------------------------|----------------|------|------|----------|------------------|
|                               |                |      |      | OD=1     | amma<br>Dmin+0.1 |
| 60 seconds<br>23° C. Water    | 6              | 1.54 | 0.08 | 3.68     | 0.18             |
| 60 seconds<br>23° C. methanol | 8              | 1.67 | 0.08 | 3.81     | 0.47             |

The vehicle was prepared by emulsion polymerization of methacrylonitrile. A vesicular coating mixture and films were prepared in generally the same manner as described in Example I. The film thus obtained was immersed for 60 seconds in 30° C. water and dried with tissue paper. Another film was immersed for 60 seconds in 30° C. methanol and dried likewise. Equilibration was accomplished in the ambient atmosphere in about one-half hour. These films were then exposed, developed, and measured as described in Example I with the following results:

60

| Treatment                     | Visbl<br>Steps | Dmax | Dmin | Speed at |                  |
|-------------------------------|----------------|------|------|----------|------------------|
|                               |                |      |      | OD=1     | amma<br>Dmin+0.1 |
| 60 seconds<br>30° C. water    | 3              | 0.75 | 0.07 | 2.67     | —                |
| 60 seconds<br>30° C. methanol | 9              | 1.43 | 0.10 | 1.94     | 0.34             |

6

A substantial improvement in photographic characteristics was obtained for the methanol treated sample, notably, threshold speed was increased by 3.5 times.

## EXAMPLE III

Vesicular films were prepared from the following formula:

| Function   | Component                                    | Parts by Weight |
|------------|----------------------------------------------|-----------------|
| Vehicle    | Methacrylonitrile-methacrylic acid copolymer | 2               |
| Sensitizer | Andrews Diazo No. 9                          | 0.08            |
| Surfactant | Disperse-Ayd No. 6                           | 0.02            |
| Solvent    | MEK                                          | 8               |
| Solvent    | Dimethyl formamide (DMF)                     | 1               |
| Solvent    | Tetrahydrofuran (THF)                        | 0.4             |

Photographic characteristics for the methanol treated sample were improved over those for the water treated film, viz, maximum density was increased, speed at optical density of 1 was 2 times faster, and threshold speed was increased by 1.7 times.

## EXAMPLE IV

Vesicular films were prepared from the following formula:

| Function   | Component                                                | Parts by Weight |
|------------|----------------------------------------------------------|-----------------|
| Vehicle    | Methacrylonitrile-2-hydroxy-ethyl methacrylate copolymer | 2.5             |
| Sensitizer | Andrews Diazo No. 9                                      | 0.1             |
| Surfactant | L-540                                                    | 0.05            |
| Solvent    | Acetonitrile                                             | 10              |
| Solvent    | 2-Methoxyethanol                                         | 2.85            |

The vehicle was prepared by emulsion copolymerization of methacrylonitrile and 2-hydroxyethyl methacrylate in a 75/25 weight ratio. L-540 is a Union Carbide silicone surfactant. The diazo compound was dis-

5 The vehicle was prepared by emulsion copolymerization of methacrylonitrile and 2-hydroxyethyl methacrylate in a 90/10 weight ratio. The formula was prepared essentially as described in Example IV and films prepared as described in Example I. The vesicular film thus obtained was immersed for 30 seconds in ambient (23° C.) water and dried with tissue paper. Another film was immersed for 30 seconds in ambient (23° C.) 10 methanol and dried as above. Equilibration was accomplished in the ambient atmosphere in about ½ hour. The two films were then exposed and developed as described in Example I with the following results:

| Treatment                  | Visbl Steps | Dmax | Dmin | Speed at OD=1 | Speed at Dmin+0.1 |
|----------------------------|-------------|------|------|---------------|-------------------|
| 30 seconds 23° C. water    | 6           | 0.13 | 0.07 | —             | —                 |
| 30 seconds 23° C. methanol | 9           | 1.37 | 0.06 | 1.71          | 0.30              |
|                            |             |      |      |               | 0.96              |

solved in 0.7 parts of 2-methoxyethanol; to this stirring solution was added the L-540 as a 25 percent solution in 2-methoxyethanol. This mixture was then added to a stirring solution of the copolymer in the remaining solvents. Vesicular films were prepared as described in Example I. 25

A film thus obtained was immersed for 60 seconds in ambient (23° C.) water and dried with tissue paper. Another film was immersed in ambient (23° C.) methanol and dried with tissue paper. Equilibration was accomplished in the ambient atmosphere in about ½ hour. The films were exposed and developed as described in Example I with the following results:

| Treatment                  | Visbl Steps | Dmax | Dmin | Speed at OD=1 | Speed at Dmin+0.1 |
|----------------------------|-------------|------|------|---------------|-------------------|
| 60 seconds 23° C. water    | 9           | 1.60 | 0.06 | 8.58          | 0.20              |
| 60 seconds 23° C. methanol | 13          | 1.35 | 0.18 | 1.13          | 0.38              |
|                            |             |      |      |               | 1.32              |

Gamma for the methanol treated sample was substantially reduced, speed at OD of 1 was increased by a factor of 1.5, and speed at the threshold level was increased by a factor of 2.6.

### EXAMPLE V

Vesicular films were prepared from the following formula:

| Function   | Component                                                | Parts by Weight |
|------------|----------------------------------------------------------|-----------------|
| Vehicle    | Methacrylonitrile-2-hydroxy-ethyl methacrylate copolymer | 2.5             |
| Sensitizer | Andrews Diazo No. 9                                      | 0.1             |
| Surfactant | L-540                                                    | 0.05            |
| Solvent    | Acetonitrile                                             | 6               |
| Solvent    | MEK                                                      | 6               |
| Solvent    | 2-Methoxyethanol                                         | 0.85            |

The vehicle was the same as described in Example V. The formula was prepared essentially as described in Example IV and films prepared therefrom as described in Example I. A vesicular film thus obtained was immersed for 60 seconds in 40° C. water and dried with tissue paper. Another film was immersed for 60 seconds in 40° C. methanol and dried as above. Equilibration was accomplished in the ambient atmosphere in about ½ hour. The thus treated films were then exposed and developed as described in Example I, with the following results:

| Treatment                  | Visbl Steps | Dmax | Dmin | Speed at OD=1 | Speed at Dmin+0.1 |
|----------------------------|-------------|------|------|---------------|-------------------|
| 60 seconds 40° C. water    | 8           | 1.61 | 0.05 | 2.61          | 0.45              |
| 60 seconds 40° C. methanol | 14          | 1.63 | 0.08 | 2.37          | 0.68              |
|                            |             |      |      |               | 1.12              |

65 Photographic characteristics for the methanol treated film were improved, especially in speed, viz, at OD of 1 speed was increased by a factor of 1.7 and at the threshold level by a factor of 2.

### EXAMPLE VII

Vesicular films were prepared from the following formula:

| Function   | Component           | Parts by Weight |
|------------|---------------------|-----------------|
| Vehicle    | Formvar 7/95S       | 2.4             |
| Sensitizer | Andrews Diazo No. 9 | 0.096           |
| Surfactant | Disperse-Ayd No. 6  | 0.048           |
| Solvent    | Ethylene Dichloride | 18              |
| Solvent    | 2-Methoxyethanol    | 0.8             |

Formvar 7/95S is a poly(vinyl formal) made by Monsanto Chemical. The diazo compound was dissolved in the 2-methoxyethanol and to this was added the Disperse-Ayd No. 6 as a 10 percent solution in ethylene dichloride. This mixture was then added to the stirring solution of the Formvar in the remaining ethylene dichloride. Films were prepared as described in Example I. A vesicular film thus obtained was immersed for 60 seconds in 30° C. water and dried with tissue paper. Another film was immersed for 60 seconds in 30° C. methanol and dried as above. Equilibration was accomplished in the ambient atmosphere in about ½ hour. These films were exposed and developed as described in Example I with the following results.

| Treatment                     | Visbl<br>Steps | Dmax | Dmin | Speed at     |                  |
|-------------------------------|----------------|------|------|--------------|------------------|
|                               |                |      |      | OD=1<br>amma | Dmin+0.1<br>amma |
| 60 seconds<br>30° C. water    | 6              | 1.58 | 0.07 | 3.20         | 0.29             |
| 60 seconds<br>30° C. methanol | 8              | 1.68 | 0.10 | 2.06         | 0.89             |

Photographic characteristics for the sample treated with methanol were greatly improved over those for the sample treated with water. Maximum density was increased and gamma reduced. Speed at OD=1 was increased by a factor of 4 and at the threshold by a factor of 8.5.

Improvement in photographic characteristics was obtained for the methanol treated film; water treatment had little effect.

#### EXAMPLE IX

Vesicular films were prepared from the following formula:

| Function   | Component           | Parts by Weight |
|------------|---------------------|-----------------|
| Vehicle    | Saran F120          | 4               |
| Sensitizer | Andrews Diazo No. 9 | 0.16            |
| Solvent    | MEK                 | 21              |
| Solvent    | 2-Methoxyethanol    | 1               |

Saran F120 is a copolymer of vinylidene chloride and acrylonitrile made by Dow Chemical. The formula was prepared by adding a solution of the diazo compound in 2-methoxyethanol to the stirring solution of the Saran F120 in MEK. Films were prepared as described in Example I. A vesicular film thus obtained was im-

mersed for 30 seconds in 40° C. water and dried with tissue paper. Another film was immersed for 30 seconds in 40° C. methanol and dried as above. Equilibration was accomplished in the ambient atmosphere in about 16 hours. The films were exposed and developed as described in Example I with the following results:

| Treatment                     | Visbl<br>Steps | Dmax | Dmin | Speed at     |                  |
|-------------------------------|----------------|------|------|--------------|------------------|
|                               |                |      |      | OD=1<br>amma | Dmin+0.1<br>amma |
| 30 seconds<br>40° C. water    | 2              | 1.15 | 0.05 | 8.58         | 0.02             |
| 30 seconds<br>40° C. methanol | 6              | 1.63 | 0.05 | 5.00         | 0.25             |

#### EXAMPLE VIII

Vesicular films were prepared from a formula as described in Example VII, except that L-540 surfactant was substituted for the Disperse-Ayd No. 6. A film thus obtained was immersed for 30 seconds in ambient (23° C.) water and dried with tissue paper. Another film was immersed for 30 seconds in ambient methanol and dried. Equilibration was accomplished in the ambient atmosphere in about ¼ hour. The films were exposed and developed as described in Example I with the following results:

The film was essentially unaffected by the water treatment. Greatly improved photographic characteristics were obtained for the sample treated with methanol.

#### EXAMPLE X

Ethyl alcohol is also effective in improving photographic characteristics as shown in this example. Films as described in Example I were immersed for 30 seconds in 40° C. water and in 40° C. ethanol and dried

| Treatment                     | Visbl<br>Steps | Dmax | Dmin | Speed at     |                  |
|-------------------------------|----------------|------|------|--------------|------------------|
|                               |                |      |      | OD=1<br>amma | Dmin+0.1<br>amma |
| 30 seconds<br>23° C. water    | 3              | 0.91 | 0.07 | 3.64         | —                |
| 30 seconds<br>23° C. methanol | 7              | 1.67 | 0.12 | 6.00         | 0.30             |

with tissue paper. Equilibration was accomplished in the ambient atmosphere in about 7 hours and 24 hours, respectively. After exposure and development as described in Example I, the following results were obtained:

| Treatment                    | Visbl<br>Steps | Dmax | Dmin | Speed at     |          |
|------------------------------|----------------|------|------|--------------|----------|
|                              |                |      |      | OD=1<br>amma | Dmin+0.1 |
| 30 seconds<br>40° C. water   | 3              | 1.72 | 0.08 | 23           | 0.22     |
| 30 seconds<br>40° C. ethanol | 6              | 1.72 | 0.08 | 4.45         | 0.54     |
|                              |                |      |      |              | 0.78     |

Gamma was greatly reduced and speed increased substantially with ethanol treatment; photographic speed at OD=1 was two times faster and at the threshold level 2.8 times faster than for the water treated film.

#### EXAMPLE XI

Combining a methanol treatment with a follow-up water treatment greatly reduces the time required to sensitize a vesicular film as shown in this example. Vesicular films were prepared from a formula similar to that described in Example IV, except that the copolymer was a 94/6 by weight methacrylonitrile-2-hydroxyethyl methacrylate. Films were prepared as described in Example I. A vesicular film thus obtained was immersed in ambient (23° C.) water for 7 minutes and dried with tissue paper. Equilibration was accomplished in the ambient atmosphere in about 72 hours. A second film was immersed for 10 seconds in 30° C. methanol, removed, and immediately immersed for 30

In Examples XII, XIII and XIV, exposure and development conditions were:

#### 1. Resolution:

USAF 8007N target; 1½ seconds, 6 inches distance with the III Hg lamp.

#### 2. Density:

Kodak Photographic Step Wedge; 60 seconds, 3½ inches distance (from heat shield) with Hanovia Hg lamp. Development Temperature = 127° C.

#### EXAMPLE XII

This example further illustrates the effectiveness of the preferred two-step alcohol-water treatment on a vesicular film. In this case the vesicular film was the same as in Example VII except that it did not contain any surfactant. Equilibration was accomplished in the ambient atmosphere in about 72 hours and 16 hours, respectively. Treatment conditions and film performance were as follows:

| Treatment                      | Visbl<br>Steps | Dmax | Dmin | Speed at     |          |
|--------------------------------|----------------|------|------|--------------|----------|
|                                |                |      |      | OD=1<br>amma | Dmin+0.1 |
| 5 seconds<br>40° C. methanol + |                |      |      |              |          |
| 30 seconds<br>23° C. water     | 7              | 1.37 | 0.07 | 3.53         | 0.20     |
| 30 seconds<br>40° C. water     | 4              | 1.32 | 0.05 | 5.00         | 0.12     |
|                                |                |      |      |              | 0.35     |

seconds in ambient water, then dried with tissue paper. Equilibration was accomplished in the ambient atmosphere in over ½ hour. A third film was immersed for 5 seconds in 40° C. methanol, removed, and immediately immersed for 30 seconds in ambient water, then dried with tissue paper. Equilibration was accomplished in the ambient atmosphere in over ½ hour. The films were exposed for 30 seconds and developed at 120° C. in the manner described in Example I with the following results:

| Treatment                                                     | Visbl<br>Steps | Dmax | Dmin | Speed at     |          |
|---------------------------------------------------------------|----------------|------|------|--------------|----------|
|                                                               |                |      |      | OD=1<br>amma | Dmin+0.1 |
| 7 minutes<br>23° C. water                                     | 8              | 1.30 | 0.09 | 2.14         | 0.44     |
| 10 seconds<br>30° C. methanol<br>plus 30 seconds<br>23° water | 14             | 1.43 | 0.11 | 2.14         | 0.70     |
| 5 seconds<br>40° C. methanol<br>plus 30 seconds<br>23° water  | 14             | 1.40 | 0.19 | 1.36         | 0.81     |
|                                                               |                |      |      |              | 1.70     |

#### EXAMPLE XIII

This example illustrates the effectiveness of an alkanol treatment where the alkanol is isopropanol. The vesicular film employed was the same as that in Example I. The equilibration time for all samples was about 7 hours exposure to ambient atmosphere. The performance of such a film treated with isopropanol under the conditions shown as follows:

| Treatment                  | Visbl<br>Steps | Dmax | Dmin | Speed at     |          |
|----------------------------|----------------|------|------|--------------|----------|
|                            |                |      |      | OD=1<br>amma | Dmin+0.1 |
| 30 seconds<br>40° C. IPA   | 4              | 1.68 | 0.08 | 10.0         | 0.22     |
| 30 seconds<br>40° C. IPA + |                |      |      |              |          |
| 15 seconds<br>23° C. water | 3              | 1.70 | 0.08 | 10.0         | 0.22     |
| 30 seconds<br>40° C. water | 3              | 1.72 | 0.08 | 23.0         | 0.22     |
|                            |                |      |      |              | 0.34     |

#### EXAMPLE XIV

This example illustrates the effectiveness of acetonitrile in treating a vesicular film having a poly(hydroxyether) polymer of the type previously described. In this example the vehicle was the same as that in Example

A substantial reduction in film treatment time is effected by the methanol-water method accompanied by significant increases in photographic speed. Speed at OD of 1 is increased by factors of 1.8 and 2.3, and at threshold by factors of 3 and 6.5.

I with the formulation containing a fluorocarbon surfactant of the type described in the above-referenced U.S. Pat. application Ser. No. 55,976. The film was treated in 23° C. acetonitrile for 15 and 30 seconds with and without a second stage water treatment at 23° C. A haze developed during the acetonitrile development within 15 seconds which completely disappeared within two minutes upon exposure to air. Exposure to air was continued for a total of 18 hours. A comparison

5

10

## EXAMPLE XVI

This example illustrates the long term effect of the treatment provided by this invention. A vesicular film as described in Example I was treated with methanol in accordance with this invention. Another sample was treated with water. Exposure and development 8½ months after treatment (during which time equilibration with the ambient atmosphere occurred) in accordance with the conditions in Example XV gave the following results:

| Treatment                     | Visbl<br>Steps | Dmax | Dmin | Speed at |      |          |
|-------------------------------|----------------|------|------|----------|------|----------|
|                               |                |      |      | OD=1     | amma | Dmin+0.1 |
| 30 seconds<br>23° C. methanol | 9              | 1.66 | 0.07 | 3.20     | 0.52 | 0.92     |
| 30 seconds<br>85° C. water    | 8              | 1.61 | 0.08 | 3.33     | 0.42 | 0.96     |

was made with the same film which received only a water treatment under the conditions stated. The performance of the treated film is as follows.

20

| Treatment                                                              | Resl<br>1/mm | Visbl<br>Steps | Dmax | Dmin | Gamma | Speed at |          |
|------------------------------------------------------------------------|--------------|----------------|------|------|-------|----------|----------|
|                                                                        |              |                |      |      |       | OD=1     | Dmin+0.1 |
| 15 seconds<br>23° C. aceto-<br>nitrile                                 | 128          | 6              | 1.60 | 0.06 | 4.00  | 0.49     | 0.73     |
| 15 seconds<br>23° C. aceto-<br>nitrile + 15<br>seconds 23° C.<br>water | 144          | 6              | 1.60 | 0.06 | 4.00  | 0.49     | 0.73     |
| 30 seconds<br>23° C. aceto-<br>nitrile                                 | —            | 7              | 1.57 | 0.06 | 2.96  | 0.49     | 0.84     |
| 30 seconds 23° C.<br>acetonitrile +<br>30 seconds 23° C.<br>water      | 203          | 8              | 1.56 | 0.06 | 3.18  | 0.47     | 0.83     |
| 15 seconds<br>85° C. water                                             | 102          | 7              | 1.68 | 0.06 | 4.38  | 0.57     | 0.86     |
| 30 seconds<br>85° C. water                                             | 102          | 7              | 1.70 | 0.07 | 4.12  | 0.63     | 0.93     |

## EXAMPLE XV

This example further illustrates the effectiveness of the present treatment where the vesicular film formulation does not contain a surfactant. In this example the film employed was the same as that in Example I except that no surfactant was added. The film was treated for 15 seconds in ambient, i.e., about 23° C. methanol. The treatment produced a light fog to moderate fog which cleared to a very light fog within ½ hour after treatment. Comparative samples of the same film were also treated for 15 seconds in 85° C. water; no fog developed. Both samples were equilibrated with the ambient atmosphere for 18 hours. Exposure and development conditions were: 60 seconds exposure through a Kodak Photographic Step Wedge No. 3 and 3½ inches distance from the Hanovia Hg arc lamp (distance from heat shield). Development temperature = 110° C.

Exposed and developed films were measured on a MacBeth TD205 Densitometer. Characteristic curves gave the following data:

The film sample identified as Eponol 55 was prepared as in Example I except that no surfactant was added to the formulation where indicated and the Union Carbide fluorocarbon surfactant FC-170 was substituted for the silicones of Example I in the other instances.

The film sample identified as Saran F-120 was prepared as in Example IX but no surfactant was used in the formulation.

Treatment was accomplished by placing the film in vapor over a heated liquid bath. Time of exposure and temperatures of the vapor and liquid baths are shown in the table below. The vapor temperature was measured about 7 inches above the liquid and is therefore cooler than the vapor closer to the liquid surface.

The acetonitrile vapor treated samples were exposed and developed as in the preceding examples between 19 and 21½ hours after treatment to effect equilibration. The methanol vapor treated samples were equilibrated with the ambient atmosphere between 17 and 18 hours before the same exposure and development.

| Treatment                     | Visbl<br>Steps | Dmax | Dmin | Speed at |      |          |
|-------------------------------|----------------|------|------|----------|------|----------|
|                               |                |      |      | OD=1     | amma | Dmin+0.1 |
| 15 seconds<br>23° C. methanol | 8              | 1.40 | 0.08 | 3.75     | 0.32 | 0.76     |
| 15 seconds<br>85° C. water    | 4              | 0.31 | 0.08 | —        | —    | —        |

Results are shown in the following table. Density values are not strictly comparable to the preceding examples. Values are higher due to changes in the densitometers used for the measurements.

ated with liquid methanol. After eight minutes of equilibration the film was exposed and developed as in the preceding examples. No image was observed. It is estimated from a curve developed from the data in the

## SENSITOMETRIC PROPERTIES

| Sample                    | Treatment                           | No. of Visible 0.15 Steps | Speed at         |                  |          |                         |      |
|---------------------------|-------------------------------------|---------------------------|------------------|------------------|----------|-------------------------|------|
|                           |                                     |                           | D <sub>max</sub> | D <sub>min</sub> | $\gamma$ | D <sub>min</sub> + 0.10 | 1.00 |
| <u>Acetonitrile Vapor</u> |                                     |                           |                  |                  |          |                         |      |
| Eponol 55/no surfactant   | NONE                                | 2                         | 2.15             | 0.13             | 5.90     | 0.29                    | 0.18 |
| do.                       | 30 seconds at 41°C (liquid at 75°C) | 6                         | 2.60             | 0.13             | 5.35     | 0.75                    | 0.59 |
| do.                       | 5 seconds at 42°C (liquid at 74°C)  | 5                         | 2.58             | 0.13             | 5.70     | 0.69                    | 0.54 |
| Eponol 55/FC-170          | NONE                                | 3                         | 2.40             | 0.14             | 5.00     | 0.48                    | 0.34 |
| do.                       | 30 seconds at 40°C (liquid at 73°C) | 6                         | 2.62             | 0.14             | 5.00     | 0.80                    | 0.63 |
| do.                       | 5 seconds at 42°C (liquid at 74°C)  | 6                         | 2.58             | 0.14             | 4.55     | 0.81                    | 0.64 |
| <u>Methanol Vapor</u>     |                                     |                           |                  |                  |          |                         |      |
| Eponol 55/no surfactant   | 30 seconds at 41°C (liquid at 51°C) | 5                         | 2.60             | 0.13             | 5.00     | 0.79                    | 0.61 |
| do.                       | 15 seconds at 60°C (liquid at 65°C) | 6                         | 2.61             | 0.14             | 4.60     | 0.76                    | 0.54 |
| Eponol 55/FC-170          | 30 seconds at 44°C (liquid at 53°C) | 7                         | 2.62             | 0.14             | 3.70     | 0.97                    | 0.79 |
| do.                       | 15 seconds at 60°C (liquid at 65°C) | 7                         | 2.56             | 0.25             | 3.65     | 1.06                    | 0.74 |
| Saran F-120/no surfactant | NONE                                | 3                         | 1.68             | 0.13             | 4.00     | 0.31                    | 0.18 |
| do.                       | 30 seconds at 38°C (liquid at 50°C) | 6                         | 2.46             | 0.17             | 3.65     | 0.78                    | 0.61 |
| do.                       | 15 seconds at 61°C (liquid at 65°C) | 6                         | 2.46             | 0.13             | 3.55     | 0.79                    | 0.58 |

## EXAMPLE XVIII

This example illustrates the relationship between 30 time and extent of solvent loss during equilibration and the necessity of an adequate equilibration period so that sufficient solvent is released.

The Eponol 55 film of the preceding Example XVII was treated with liquid phase methanol and vapor phase acetonitrile. The following table shows the decrease in solvent retention with equilibration time for the two treatments.

above table that the film had a retained solvent content of about 5% based on the coating weight.

Similarly the same film was treated with acetonitrile vapor and exposed and developed 1½ hours after treatment. Only three steps were observed with no image appearing in the portion of the film receiving the greater vapor treatment. It is estimated from a curve developed from the data in the above table that the film had a 5 percent retained solvent content based upon the coating weight.

## SOLVENT WEIGHT LOSS MEASUREMENTS

| Equilibration Time, Hours                                                          | Sample wt. (including polyester base), g. | Wt. of retained Solvent, g. | % Solvent Retention Based on Coating Weight |
|------------------------------------------------------------------------------------|-------------------------------------------|-----------------------------|---------------------------------------------|
| Liquid Methanol Treatment [Actual coating wt. (minus base film) = 0.0804 gram.]    |                                           |                             |                                             |
| Before treatment                                                                   | 1.6596                                    | —                           | —                                           |
| 0                                                                                  | 1.6692                                    | 0.0096                      | 11.95                                       |
| 0.25                                                                               | 1.6629                                    | 0.0033                      | 4.10                                        |
| 0.50                                                                               | 1.6605                                    | 0.0009                      | 1.12                                        |
| 0.75                                                                               | 1.6600                                    | 0.0004                      | 0.50                                        |
| 1.00                                                                               | 1.6597                                    | 0.0001                      | 0.125                                       |
| Acetonitrile Vapor Treatment [Actual Coating wt. (minus base film) = 0.0937 gram.] |                                           |                             |                                             |
| Before treatment                                                                   | 1.7165                                    | —                           | —                                           |
| 0                                                                                  | 1.7260                                    | 0.0095                      | 10.10                                       |
| 0.30                                                                               | 1.7236                                    | 0.0071                      | 7.58                                        |
| 1.00                                                                               | 1.7224                                    | 0.0059                      | 6.30                                        |
| 1.50                                                                               | 1.7209                                    | 0.0044                      | 4.70                                        |
| 3.00                                                                               | 1.7196                                    | 0.0031                      | 3.31                                        |
| 4.00                                                                               | 1.7196                                    | 0.0031                      | 3.31                                        |
| 6.00                                                                               | 1.7187                                    | 0.0022                      | 2.35                                        |
| 22.00                                                                              | 1.7178                                    | 0.0013                      | 1.39                                        |
| 24.00                                                                              | 1.7176                                    | 0.0011                      | 1.17                                        |
| 30.00                                                                              | 1.7171                                    | 0.0006                      | 0.64                                        |

Where equilibration has not proceeded for a sufficient period of time and a substantial portion of the solvent is still contained in the film, the photographic properties of the film may be impaired to the point that the film is useless. As an illustration, the film identified as Eponol 55 of this and the preceding example was tre- 65

I claim:

1. In the method for improving the photographic characteristics of vesicular film comprising a synthetic hydrophobic vehicle substantially resistant to physical degradation by lower alkanol solvents coated and dried on a support, said vehicle being of the type adapted to

serve as the vehicle for a light-sensitive material to form vesicular images, a light-sensitive material substantially uniformly dispersed in said vehicle, said light-sensitive material being decomposable to form nitrogen gas upon imagewise exposure to actinic radiation, said film being heat developable to form vesicles in the exposed areas, the improvement comprising immersing the film prior to imagewise exposure in a fluid phase alkanol having up to three carbon atoms, and thereafter equilibrating said immersed film prior to said imagewise exposure to permit release of alkanol from the film so that less than about 1 percent is retained therein, the time and temperature of said immersion and the time of said equilibration being sufficient to increase the photosensitivity of the film.

2. The method in accordance with claim 1 wherein said fluid phase is liquid.

3. The method in accordance with claim 1 wherein said fluid phase is vapor.

4. The method in accordance with claim 1 wherein said alkanol is methyl alcohol.

5. A method in accordance with claim 1 wherein said alkanol is ethyl alcohol.

6. A method in accordance with claim 1 wherein said vesicular film has as its vehicle a film forming thermoplastic linear poly (hydroxy ether) polymer of an epichlorohydrin and a dihydric phenol.

7. A method in accordance with claim 1 wherein said vesicular film has as its vehicle a copolymer of about 70-99 weight percent of a nitrile of the formula:



copolymerized through the respective ethylenically unsaturated sites with about 1-30 weight percent of a hydroxy substituted acrylate of the formula:



10 in which X and Y are individually selected from hydrogen, methyl, and chlorine.

8. A method in accordance with claim 1 and including the step of contacting said film with water after said contact with the alkanol.

9. A method in accordance with claim 1 wherein said contact with the alkanol is executed at a temperature of about 20°-60° C. for about 1-100 seconds.

10. A method in accordance with claim 8 wherein said contact with the water is executed at about 20°-90° C. for about 1-100 seconds.

11. A method in accordance with claim 8 wherein said contact with the alkanol is executed at about 20°-40° C., said contact with the water is executed at ambient temperature, and said alkanol is methyl alcohol.

12. A method in accordance with claim 6 wherein said vehicle is a polymer of epichlorohydrin and 2,2'-bis(*p*-hydroxyphenyl) propane.

13. A method in accordance with claim 7 wherein said vehicle is a polymer of methacrylonitrile and 2-hydroxyethyl methacrylate.

\* \* \* \* \*